

No. 882,720.

PATENTED MAR. 24, 1908.

M. J. SOMERS.

METHOD OF PRODUCING CHILLED CASTINGS.

APPLICATION FILED OCT. 12, 1907.

Fig. 1



Fig. 2



Fig. 3



Fig. 4



Fig. 5



WITNESSES.

George Oltach

J. M. Cole.

15 18 BY *Mitchell J. Somers*  
*Atty. to Inventor*

INVENTOR  
ATTY

# UNITED STATES PATENT OFFICE.

MITCHELL J. SOMERS, OF SOUTH BEND, INDIANA, ASSIGNOR TO SOUTH BEND FOUNDRY CO., OF SOUTH BEND, INDIANA, A CORPORATION OF INDIANA.

## METHOD OF PRODUCING CHILLED CASTINGS.

No. 882,720.

Specification of Letters Patent. Patented March 24, 1908.

Application filed October 12, 1907. Serial No. 397,196.

*To all whom it may concern:*

Be it known that I, MITCHELL J. SOMERS, a citizen of the United States, residing at South Bend, in the county of St. Joseph and State of Indiana, have invented certain new and useful Improvements in Methods of Producing Chilled Castings, of which the following is a specification.

This invention relates to methods for casting articles upon the rims of which it is desired to produce a chilled surface, and has for its object to simplify and improve the means whereby such results are accomplished.

The improved method is designed more particularly for producing a chilled rim upon the exposed upper ends of the man-hole castings which are employed at the entrance of sewers, electric conduits and the like in the pavements of streets, to provide a hard surface at the portions of such structure which are exposed to the impact of the wheels of vehicles and the hoofs of horses and the like, and for the purpose of illustration, the improved process is shown in the drawings applied to the production of a structure of this character, and in the drawings thus employed.

Figure 1 is a transverse section of a flask illustrating the first step of the process. Fig. 2 is a plan view of the parts shown in Fig. 1. Fig. 3 is a view similar to Fig. 1 illustrating the second step in the process. Fig. 4 is a view similar to Figs. 1 and 3 illustrating the third step in the process. Fig. 5 is a sectional view illustrating the 4th 5th and 6th steps in the process.

The drag or lower portion of a conventional flask is represented at 10 mounted upon the base board 11, of usual construction.

12 represents a portion of the pattern of a man-hole of conventional form, and 13 represents a pattern of a chilling element, which in this instance is in the form of an annular rim, and attached to this chilling element pattern is the remaining portion of the pattern and represented at 14, in this instance in the form of an annular rib which bears against the inner surface of the upper portion of the pattern 12.

The molding sand is indicated at 15, and is tamped around the patterns 12—13—14, as represented in Fig. 1, which illustrates the

first step in the improved process. After 55 the tamping is completed the pattern 13 of the chilling element, together with its pattern portion 14, is removed, leaving the annular cavities 16—17, as indicated in Fig. 3, which represents the second step in the improved process.

A chilling element which in this instance is in the form of an annular ring 18, is then inserted into the cavity 16, leaving the cavity 17 vacant, as illustrated in Fig. 4, which represents the third step in the improved process. The flask 10, with its contents, is then inverted, as illustrated in Fig. 5, and the main pattern portion 10 removed in the ordinary manner, leaving the complete space, 70 including the cavity 17, vacant, as shown. The cope member 19, having therein suitable sprues 20, is then disposed over the flask 10, as shown in Fig. 5, which represents the fifth step in the improved process. The flask and 75 its cope are now in condition to receive the molten metal, which is poured through the sprues 20 in the ordinary manner and completes the various steps of the process. The molten metal, it will be obvious, which 80 comes in contact with the element 18, will be "chilled" or hardened.

The cavity 17 it will be noted, forms an annular rib spaced from the adjacent edge of the casting when completed, and the chilling 85 element 18 is formed with sharply defined corners over which the molten metal is chilled, and correspondingly sharply defined corners are produced in the casting at the juncture of the upper face of the rib there- 90 with, as will be obvious. In forming castings of the character shown in the ordinary manner, by employing ordinary wooden patterns, the molten metal is liable to distort the relative soft molding sand at the corners of the 95 rib and produce uneven surfaces, which require to be removed by chipping or otherwise before the covers can be placed in position. This is an expensive and troublesome necessity and is entirely avoided by the improved 100 process herein described, wherein the relatively sharp corner at the juncture of the rib and wall of the casting is reproduced in the casting, thereby obviating the necessity for chipping or otherwise treating the casting 105 after it leaves the sand. This is an important feature of the improved process, and adds materially to the value and utility

thereof. In devices of the character shown, wherein the upper edges are exposed to the heavy friction incident to the traffic passing over them, the hardening of the exposed 5 portions is very desirable, and the improved process herein described produces this hardened surface in a very simple and inexpensive manner. It will be noted that in producing the improved casting, the flask 10 requires to be inverted but once, and the employment of the chilling element 18 materially lessens the number of manipulations of the flask, which would otherwise be required 10 to form a mold of the same design. Man-hole 15 castings of the character described weigh from 250 to 350 pounds, besides the weight of the flask and the molding sand, consequently the less handling is required in forming the mold is important, as will be obvious, 20 to say nothing of the liability to injury of the mold during the formation.

What is claimed is—

The method of producing castings having a chilled rim consisting; first, in tamping in a flask a pattern of a portion of the article to be cast, together with a pattern of a chilling element having connected thereto the remainder of the article to be cast; second, removing the pattern of the chilling element and its said attached pattern portion; third, 25 inserting a chilling element into the cavity formed by the removal of the chilling element pattern; fourth, removing the first mentioned pattern portion; fifth, placing a cope element having suitable sprues upon the 30 flask; sixth, inserting the molten metal.

In testimony whereof I affix my signature, in presence of two witnesses.

MITCHELL J. SOMERS.

Witnesses:

F. E. BURGENER,  
GEORGE OLTSCHE.